

Patented Nov. 14, 1922.

## UNITED STATES PATENT OFFICE.

ROBERT ABBOTT HADFIELD, OF WESTMINSTER, ENGLAND.

## MANUFACTURE OF STEEL.

No Drawing. Application filed July 15, 1916, Serial No. 109,436. Renewed February 11, 1921. Serial No. 444,305.

*To all whom it may concern:*

Be it known that I, Sir ROBERT ABBOTT HADFIELD, F. R. S., a subject of the King of Great Britain and Ireland, residing at Westminster, England, have invented new or improved Manufacture of Steel, of which the following is a specification.

This invention has for its object the manufacture of a manganese steel or iron alloy possessing amongst other qualities, great toughness and resistance to perforation, particularly when in the form of heat treated sheets or plates.

I have found that this object can be attained by using an alloy of iron, carbon, silicon, manganese and copper. The copper may be added to an alloy of iron, carbon, silicon and manganese of the kind ordinarily known as manganese steel which usually contains a small percentage of silicon, seldom exceeding 3%. When the desired percentage of silicon in an alloy of this kind is not sufficiently high for any desired alloy according to the invention, and usually 25 a higher percentage, say from about .6 to 2% will be necessary to obtain the best results, additional silicon must be added to the alloy referred to in addition to the copper. Such a percentage of silicon is relatively 30 high in relation to that usually existing in ordinary manganese steel.

The new alloy of iron, carbon, silicon, manganese and copper which forms a new manganese steel, may vary in the percentage 35 composition of its constituents, but the percentage of manganese will always be high relatively to the other constituents except the iron. It may for example comprise iron with about from .9 to 2% of carbon, with 40 from about .1 to 2% or above of silicon, with from about 10 to 15% or it may be up to 17% of manganese and from about 1 to 3 or 4% of copper, but the invention is not limited to these percentages, the main feature of the new steel or alloy being the presence therein of silicon and copper. The 45 copper, and also the silicon, when an additional quantity thereof is used, may be added to ordinary manganese steel when in the molten state, or to the mixture of iron and ferro-manganese, or iron and manganese, used to produce such ordinary manganese steel, and melted simultaneously therewith, the resulting new manganese steel 50 being cast into ingots or other castings. The

copper may be added as such, or in any other suitable form. When additional silicon is used, it may be added as such or in any other suitable or convenient form, as for example 60 ferro-silicon or silicon spiegel.

The quality of the new manganese steel or iron alloy can be improved, at least for some purposes, by subjecting it to a toughening process consisting in heating it to a high 65 temperature, say for example to about 900° C. and up to it may be 1050° C. or above but below its melting point, and cooling it quickly, as by quenching it in water. The new steel or alloy when thus heat treated 70 and water quenched, usually called water toughened, has a greater toughness and resistance to perforation than ordinary manganese steel of commerce.

For many purposes, the new steel or alloy 75 may advantageously be rolled into the form of sheets or plates (hereinafter referred to as sheets), or of rods, bars or wire, and be subjected to the toughening process referred to, when in such form, or previously, as when 80 in the form of ingots or slabs. If desired, the toughening process may be repeated. The new steel or alloy can also be used for castings of any desired shape and be heat treated or not as may be required.

Another element, such for example as 85 chromium, nickel, cobalt, vanadium, tungsten, titanium or aluminium, or two or more of such elements, may be added to the new steel or alloy for the purpose of improving 90 or varying the quality thereof. The percentage of such element or elements employed is such as to give to the resulting steel or iron alloy the varying desired qualities.

By way of example, it may be stated that 95 good results have been obtained with a steel or iron alloy according to the invention and in the form of water toughened plates or sheets, when containing about .95% of carbon, about 1.25% of silicon, about 12.72% of manganese and about 1.44% of copper and also with a steel or iron alloy containing about 1.24% of carbon, about .11% silicon, 100 about 12.42% of manganese and about 1.18% of copper.

The new steel or iron alloy can be used for 105 various purposes and in either the rolled, forged or cast condition.

What I claim is:—

1. A steel alloy containing from about

- two per cent and upwards of manganese, from about seven tenths per cent up to about two per cent of carbon, a substantial amount of copper, and from one tenth per cent and 5 upwards of silicon.
2. A steel alloy containing from about ten per cent and upwards of manganese, carbon up to two per cent, copper up to four per cent and silicon up to two per cent.
- 10 3. A steel alloy containing from about ten per cent and upwards of manganese, from about one to four per cent of copper and from about one tenth per cent to about two per cent of silicon.
- 15 4. A steel alloy containing from about ten per cent and upwards of manganese, from about seven tenths per cent to two per cent of carbon, from about one to four per cent of copper and from about one tenth 20 per cent to about two per cent of silicon.
5. A steel alloy containing over ten per cent of manganese, over one per cent of copper and from one tenth of one per cent to about two per cent of silicon.
- 25 6. A steel alloy containing over ten per cent of manganese, over one per cent of copper and a substantial amount of silicon.
7. A steel alloy having great resistance to 30 perforation and great toughness, and containing from about one tenth of one per cent to about two per cent of carbon, from about ten to about seventeen per cent of manganese, from about one to about four per cent of copper, and from about one tenth 35 of one per cent to about two per cent of silicon.
8. A steel alloy containing from about twelve to thirteen per cent of manganese, from about nine tenths per cent to about one 40 decimal five per cent of carbon, from about one per cent to one decimal five per cent of copper, and from about one tenth per cent to about one decimal five per cent of silicon.
9. Manganese steel containing from about 45 one to four per cent of copper and a substantial amount of silicon.
10. A steel alloy containing manganese from about ten per cent and upwards, carbon up to about two per cent, copper up to 50 four per cent and silicon up to two per cent and treated by heat above about 900° C. and below its melting point and then cooled quickly.
11. As a new article of manufacture, manganese steel in wrought form, having great 55 toughness and resistance to perforation and containing from one to four per cent of copper and a substantial amount of silicon.
12. As a new article of manufacture, manganese steel in sheet form, having great 60 toughness and resistance to perforation and containing from about one to four per cent of copper and a substantial amount of silicon.
13. A steel alloy containing carbon from 65 about .9 to about 1.50 per cent, manganese from about ten to about seventeen per cent, copper from about one to about four per cent and silicon from about one tenth per cent to about two per cent, and treated by heat 70 above about 900° C. and below its melting point, and then cooled quickly.
14. As a new article of manufacture, steel having great toughness and resistance to 75 perforation and containing from about ten to seventeen per cent of manganese, from about seven tenths per cent to one and five tenths per cent of carbon, a substantial amount of copper and from about five tenths 80 per cent to two per cent of silicon.
15. As a new article of manufacture, manganese steel in wrought form and alloyed with from about one to four per cent of copper and a substantial amount of silicon 85 and treated by heat to above about 900° C. and below its melting point and then cooled quickly.
16. As a new article of manufacture, manganese steel in sheet form alloyed with from 90 about one per cent to four per cent of copper and a substantial amount of silicon up to about two per cent and treated by heat to above about 900° C. and below its melting point and then cooled quickly.
17. An iron alloy containing from 10 to 95 14% of manganese, 1.00 to 1.30% of carbon, 0.35 to 0.60% of silicon, and 0.50 to 1.75% of copper.

Signed at 22 Carlton House Terrace,  
Westminster, England, this sixteenth day 100  
of June 1916.

ROBERT ABBOTT HADFIELD.

Witnesses:

WILLIAM CROSS,  
JOHN HAROLD HALLATT.